

June 23, 1942.

R. L. DOWDELL

2,287,029

## METHOD FOR MAKING SHOT

Filed Aug. 14, 1939



INVENTOR  
RALPH L. DOWDELL  
By Paul, Paul, Moore & Giere  
ATTORNEYS

## UNITED STATES PATENT OFFICE

2,287,029

## METHOD FOR MAKING SHOT

Ralph L. Dowdell, St. Paul, Minn., assignor to  
 Regents of the University of Minnesota, Minneapolis, Minn., a corporation of Minnesota

Application August 14, 1939, Serial No. 289,980

6 Claims. (Cl. 83—91)

This invention relates to a method and apparatus for the production of lead shot and more particularly to a process and apparatus for making disintegratable lead alloy shot of the type set forth in Patent 2,167,828 issued August 1, 1939.

According to the usual methods of producing shot from lead or alloys of lead containing small percentages of arsenic and/or antimony, the spherical shot is made by dropping the molten shot metal through perforations of small size. The shot metal is permitted to fall through space for a distance sufficient to cool and solidify the same, and is finally collected in a bath of water or oil at the end of its fall.

When an alloy containing a small amount of magnesium is dropped in the ordinary "shot tower" by usual procedures, the resultant shot is not of spherical configuration, but is of irregular configuration having small "tails" on the shot particles, which render the shot unsuitable for ballistic purposes.

According to the present invention, magnesium-lead alloy shot of good spherical configuration may be fabricated by a dropping procedure and it is therefore an object of the invention to provide a method of producing lead shot by dropping. It is more particularly an object of the invention to provide an apparatus for producing a lead-alloy shot of the type set forth in Patent 2,167,828 by dropping.

It is a further object of the invention to provide a shot dropping method of fabricating spherical shot of good quality composed of lead and a small percentage of magnesium.

It is also an object of the invention to provide an apparatus for fabricating spherical lead shot of good quality by dropping and more particularly it is an object of the invention to provide an apparatus for producing shot composed of lead and a small percentage of magnesium.

Other objects of the invention are those inherent in the apparatus and methods herein illustrated, described and claimed.

The method and apparatus of the present invention are illustrated with reference to the drawing in which

Figure 1 illustrates a schematic elevational view partly in section of shot dropping apparatus for carrying out the method of the present invention, and

Figure 2 is a fragmentary enlarged view partly in section of the shot dropping plate portion of the apparatus illustrated in Figure 1.

Figure 3 is a fragmentary, elevational view,

partly in section of a modified form of the apparatus.

Throughout the drawing, like characters are used to designate corresponding parts.

5 The apparatus for carrying out the method of dropping shot set forth in the present invention may consist generally of an alloying or shot metal melting arrangement represented in Figure 1 by the portion under the bracket A, in which the shot metal is melted or the lead alloy from which 10 the shot is fabricated is prepared.

According to the preferred form of the invention, the melting furnace consists of a steel or cast iron kettle 10, which is heated by any preferred means such as the electrical heating elements 11. In the shot metal melting pot illustrated, the heating element is placed in close contact with the bottom of the kettle 10, and the entire kettle and heating elements are thoroughly insulated by a thick layer of insulating material 12 which may for example be asbestos or diatomaceous earth block.

15 The molten alloy within the kettle 10 is designated 15, and in its molten state is covered by a suitable molten flux 16, which inhibits oxidation of the shot metal. In order further to reduce the possibility of oxidation, the kettle is preferably provided with a cover 17.

20 Extending from the left of the kettle 10 as shown in Figure 1, there is a steel or iron tube 20, which may be insulated, having a regulating valve 21 therein. The tube 20 extends from the shot metal melting kettle 10 to the shot dropping apparatus, which in Figure 1 is the portion under 25 the bracket B. Preferably the tube 20 and the valve 21 are covered with a thick layer of insulation which extends from the insulated kettle 10 to the insulated jacket of the shot dropping apparatus. This tube may also be an iron pipe 30 siphon elevating the molten lead alloy over the side wall of the kettle and discharging it on the shot pan 30.

25 The shot dropping apparatus, or "shot tower" consists of a shot dropping plate 30 having a plurality of apertures 31 therein. In Figure 2, which is a fragmentary enlargement of the shot dropping plate portion of Figure 1, the plate 30 is illustrated as being provided with apertures 31 having a lower cylindrical bore portion 32 and 35 an upper conical portion 33. The diameter of plate 30 may be made any dimension desired from a few inches to several feet in diameter depending upon the shot dropping capacity desired in the "shot tower," and the diameter of apertures 31 may likewise be varied according to 40 45 50 55

the size of shot which it is desired to produce. As illustrated in Figures 1 and 2, the plate 30 is held between an upper tubular portion generally designated 40 and a lower tubular portion generally designated 60, which are joined together with the plate 30 between them by means of the screw connection 41.

The plate 30 in its preferred form is nicely fitted to the tubular portion 40 at the point 42 so as to preclude flow of molten shot metal edge-wise from the plate.

The tubular portion 40 extends upwardly from the plate 30 and is provided with an outside flange 43 which serves to support tube 40 and the attached lower tubular portion 60 from the frame and jacket 69 of the apparatus. The upper end 15 of tube 40 is closed by means of a screw cap 45, through which there extends tubes 46 and 47. The tube 46 is provided with a coupling 48 by which it may be disconnected from the tube 49. It will be noted that the tube 46 in Figure 1 extends downwardly within the member 40 to within a few inches of the shot dropping plate 30. Tube 47 on the other hand communicates with the upper portion 60 of the interior of tube 40 and has an outwardly extending branch 48 adjacent which there is a pilot light 51.

The tubular portion 60 of the apparatus extends downwardly from the shot dropping plate for a distance sufficiently great that the shot dropped through the plate is spherodized before it emerges from the lower end 61. In practice, the dimension T of tube 60 is preferably made from 5 to 30 feet depending upon the temperature at which the shot is dropped and other factors, and the height H through which the shot falls is preferably made from 50 to 150 feet.

The tubular portion 60 is provided with a pipe 62, which is coupled by means of a union 63 to the pipe 64. It will be noted that pipes 48 and 64 merge at the junction 65 and are in communication with the pipe 66 which extends to a gas supply and purification apparatus, illustrated in Figure 1 under the bracket C.

The shot plate zone 30 and the adjacent portions of tubes 40 and 60 of the "shot tower" are preferably arranged to be heated so that the molten shot metal conducted to the plate 30 remains in fluid condition on top of plate 30. In the preferred form of the apparatus, the heating is accomplished by means of an electrical heating coil 70 which is fed by conductors 71 from mains 72. It is preferable to provide a variable voltage regulator 73 so that the amount of heat emitted by coils 70 may be regulated within close limits. The jacket 69 may be insulated as shown, or in some instances, it may be uninsulated.

The heating coil 70 may be used to warm the shot plate or pans at the outset of a run. Thereafter during the run the heat output of coil 70 is decreased or entirely interrupted. In some instances the coil 70 may be entirely eliminated where provision is made to heat the shot dropping plate 30 (or pans 84 where they are used) externally of the tower before the run is begun or where the shot metal is initially introduced at a sufficiently high temperature that it heats the dropping plate or pans. The coil 70 when used, permits temperature regulation to a fraction of a degree and its use is therefore desirable.

As illustrated in Figures 1 and 2, the tube 20 from the melting kettle 10 enters the shot dropping apparatus just above the plate 30 and the alloy emerging from the tube 20 thus spreads in a thin film 75 upon plate 30.

At the lower end of tube 61, there is provided a pilot light 76, which serves to burn the gas supplied to the tube 60 as hereinafter explained. At the bottom of the "shot tower" there is provided a sump 78 which is partially filled with a fluid such as carbon tetrachloride, oil or water. In the preferred form of the invention, the fluid 78 is carbon tetrachloride although when special precautions are made, other fluids such as water may be used.

The gas supply and purification apparatus illustrated under the bracket C of Figure 1, preferably consists of a gas supply bottle 80 having a shut-off valve 81, pressure gauge 82 and a pressure reduction device 83 by which the high pressure of the gas within the bottle 80 is reduced to a low constant pressure in tube 84. The gas within tube 84 is then conducted through one or more bubbling vessels 85 containing material 15 for the absorption of oxygen, and after emerging from the last bubbling vessel 85, passes through pipe 86 to a drying tower 87, which contains a material for the absorption of any water or water vapor which may be present in the gas. After passing through the drying material the gas emerges through pipe 88, which is provided with a pressure gauge 89. As explained above, the pipe 88 communicates with pipes 48 and 64 at junction 65.

In the process of producing shot according to the present invention, the shot material such as the shot alloys of Patent 2,167,828 are reduced to a molten state in kettle 10 or the alloying may be accomplished in the kettle 10 where the raw metallic materials are separately obtained. The alloying is preferably done by introducing the metallic constituents into the kettle 10 under a molten flux consisting of anhydrous, calcium chloride, magnesium chloride, barium chloride and calcium fluoride. Good results are obtained when an anhydrous flux of the following composition is used:

|                    | Per cent |
|--------------------|----------|
| Calcium chloride   | 55       |
| Magnesium chloride | 34       |
| Barium chloride    | 9        |
| Calcium fluoride   | 2        |

The alloy is melted or made by the heat supplied through heating coil 11 or by proper gas burners and after becoming thoroughly fluid is conducted through pipe 20 to the shot dropping plate 30 where it forms a thin film. The heat input to heating units 11 and 70 is adjusted so that the alloy is maintained at a temperature slightly above the temperature of solidification so that the molten shot metal accordingly drops through the holes 31 and falls through the gas atmosphere within the tube 60.

Prior to the introduction of molten shot metal above plate 30, gas is introduced into the tubes 40 and 60 by means of the gas supply and purification apparatus C. For the gas supplied in the tubes 46 and 62, there is used a substantially water and oxygen free gas which is inert to the metallic constituents of the molten shot alloy. Very excellent results are obtained when using hydrocarbon gases, more particularly the alkane gases such as "propane commercial" which is obtainable from the Mid-Continent oil fields of Oklahoma and Texas. Thus "propane commercial," or what is known in the Northwest trade as "Blaugas," gives excellent results without scrubbing oxygen and water vapor in 85 and 87. Such "bottled propane" consists predominately

of propane, about 95% to 99%, together with small percentages of other alkane gases such as methane, ethane, butane and the like. Other reducing gases inert to the molten shot metal may also be used.

When such bottled "propane, commercial" gas is used, it may be supplied in containers such as that illustrated at 80 in Figure 1 or it is also available in tank car lots. The commercial gas is relatively free of water vapor, the water having been "frozen" out in the manufacturing of the gas, and very little oxygen is normally present. However, it is preferable merely as a precaution to guard against any water and oxygen that may be present by passing the gas through the bubbling towers 85 which contain an oxygen absorption material such as pyrogallic acid, and then through the drying tower 87 which preferably contains an anhydrous strongly hygroscopic granular material such as calcium chloride.

Where the gas being used contains much moisture or oxygen, the purifying apparatus may be extended to cope with these unwanted constituents, the goal being to reduce the amount of oxygen, water vapor and the like unwanted constituents until spherical shot is obtained. The sufficiency of the purification procedure may easily be gauged by examining the shot produced, for when there is too much oxygen or water vapor slight "tails" will be formed on the spherical shot. As the oxygen and water vapor is reduced, the tails disappear, and truly spherical shot is obtained. In some instances, "propane, commercial" gas is sufficiently free of oxygen to render the pyrogallic acid oxygen scrubbers 85 unnecessary, and these may accordingly be dispensed with when the oxygen content is low or where oxygen is absent.

The purified gas is introduced into pipe 66 at a few ounces pressure and fills tubes 40 and 60.

After the gas has been passed into the tubes 40 and 60 for a period sufficient to drive out oxygen and other gaseous constituents of the atmosphere, the gas is lighted at tube 48 by means of pilot 51 and at the bottom of tube 60 by means of pilot light 76. Thereafter, throughout the dropping operation, gas is supplied to tube 40 above the shot dropping plate 30 by means of tubes 46 and to the tube 60 below the shot dropping plate by means of tube 62 and the flow of gas is burned with a quiet flame at the end of tube 40 and at the bottom of tube 61.

With the gas thus supplied to tubes 40 and 60, the molten shot metal is introduced onto the shot dropping plate 30 by way of tube 20 as previously described and the molten shot metal drops through the apertures 31 and downwardly through the tube 60.

The distance of dropping through tube 60 and the temperature within this zone is sufficiently low that by the time the shot globules drop through quiet flame at the bottom of tube 61, they have already assumed a spherical form and cooled sufficiently to resist deterioration while falling through the atmosphere to sump 78. Where the shot being dropped consists of ordinary lead or lead arsenic and lead antimony alloys, the sump 78 may contain water, but where the shot is of a disintegrable lead alloy such as that set forth in Patent 2,167,828 I prefer to use a light evaporatable fluid such as carbon tetrachloride. However, where provision is made for the immediate removal and drying of a disintegrable alloy shot collects in sump 78, water may be used as the fluid 79 even when

the shot consists of an alloy of lead and magnesium.

After the shot is removed from sump 78 and dried, it is graded by any of the usual procedures and then graphited, oiled or coated with grease or resinous material. Any malformed or imperfect shot which is separated in the grading process may be returned along with fresh material to the shot metal melting kettle 10 where it again passes through the shot forming procedure.

In carrying out the invention care should be taken to supply the molten shot metal to the plate 30 in a thin layer for if the layer 75 of shot metal on the plate 30 is increased in thickness shot of elliptical formation is likely to result.

In the modification shown in Figure 3, tube 40 is provided with a door 89, hinged at 90 to tube 40. Access to door 89 is made available by providing an opening 92 in the insulated or unin- 20 sulated jacket 69 of the shot tower. Door 90 may be provided with a glass sighting opening 91 if desired so as to enable the operator to judge the procedure of dropping. (See Figure 1.) In this modification plate 30 is provided with two or more holes 93 which are chamfered to receive shot pans 94—94. The shot pans are similar in shape to an ordinary frying pan and are of a size so that they can easily be removed through door 89 for cleaning and for changing pans to produce different "sizes" of shot. In this modification it is of course understood that each of the pans 94 has apertures in its lower 25 surface which are preferably of the shape shown at 31 in Figure 2. Only one pan is normally used at a time and the shot metal delivery tube 95 is thus made so that it can be moved from the full line position 96 where it serves the pan 94 at the right of Figure 3, to the position 97 where it serves the pan 94 at the left of Figure 3.

Many obvious variations will be apparent to those familiar with the art and may be made in the details of the apparatus and method herein described. Thus the exact proportions of the constituents in the shot metal may be widely varied although the method is especially adapted for the production of good quality spherical shot of lead and a small percentage of magnesium, and other disintegrable shot metals of the type set forth in Patent 2,167,728. Likewise, the type of gas supplied above and below the shot dropping plate may be widely varied and may include normally gaseous alkanes derived from natural sources or manufacturing operations or normally liquid hydrocarbons which are converted to the gaseous phase at the temperatures used in the dropping procedure. Variations may be made in the gas purification procedure or may be omitted entirely where the source of gas supply is assuredly substantially free of oxygen and water vapor, and other gas purification steps may be included for the removal of constituents of any selected gas which are not inert to the shot metal at the temperatures used in the dropping procedure. Likewise the method of heating the shot metal melting shot and the method of heating the "shot tower" apparatus may be varied to suit the conditions of any particular installation and the dimensions of the shot dropping plate, the size of the apertures 31, tubes 40—60 and dimensions H and T may likewise be widely varied to meet the exigencies of any particular installation. Furthermore, in some instances it is desirable to incorporate the

shot melting kettle with the "shot tower" or to use other methods than that illustrated, for example a siphon, for conducting the molten shot metal from a melting kettle to the upper surface of the shot dropping plate. These and other variations may all be made without departing from the spirit of the invention herein illustrated, described and claimed as follows:

I claim:

1. A process of making spherical shot which comprises supplying a molten alloy of  $\frac{1}{2}$  to 10% magnesium and 99 $\frac{1}{2}$  to 90% lead to the upper surface of a perforated plate for dropping therethrough, said dropping being carried out in a hydrocarbon gas which is free of water vapor and oxygen.

2. A process of making spherical shot which comprises dropping an alloy of  $\frac{1}{2}$  to 10% magnesium and 99 $\frac{1}{2}$  to 90% lead through perforations in a plate in an atmosphere of an alkane hydrocarbon gas which is free of water vapor and oxygen.

3. A process of making spherical shot which comprises dropping an alloy of  $\frac{1}{2}$  to 10% magnesium and 99 $\frac{1}{2}$  to 90% lead through a perforated plate, said dropping being carried out in an atmosphere of propane which has been freed of oxygen and water vapor.

4. A process of fabricating spherical shot

which comprises dropping an alloy comprising lead 99 $\frac{1}{2}$  to 90% and magnesium  $\frac{1}{2}$  to 10% through an orifice and maintaining a gaseous atmosphere of an alkane hydrocarbon which has been freed of oxygen and water vapor around said molten metal until after it has dropped said orifice and partially solidified.

5. A process which comprises melting an alloy of 99 $\frac{1}{2}$  to 90% lead and  $\frac{1}{2}$  to 10% magnesium under an oxidation inhibiting flux comprising a chloride of an alkali metal, transferring said molten alloy out of contact with oxygen to a plate having perforations therein for dropping the alloy therethrough, and maintaining around said molten alloy an atmosphere of propane which is free of oxygen and water vapor around said alloy during the dropping thereof.

6. A process which comprises melting an alloy of 99 $\frac{1}{2}$  to 90% lead and  $\frac{1}{2}$  to 10% magnesium under an oxidation inhibiting flux comprising a chloride of a metal selected from the group consisting of magnesium, sodium, potassium, barium and calcium, transferring said molten alloy out of contact with oxygen to a plate having perforations therein for dropping the alloy therethrough and maintaining an atmosphere of propane free of oxygen and water vapor around said alloy during dropping thereof.

RALPH L. DOWDELL.